

# United States Patent Office

3,004,850  
Patented Oct. 17, 1961

1

3,004,850

## PRODUCTION OF POSITIVE PHOTOGRAPHIC RECORDS

Harold Owen Dickinson and George Frank Duffin, Ilford, England, assignors to Ilford Limited, Ilford, England, a British company  
No Drawing. Filed Nov. 23, 1959, Ser. No. 854,614  
Claims priority, application Great Britain Nov. 28, 1958  
12 Claims. (Cl. 96—29)

This invention relates to the production of positive photographic records by the method generally known as the diffusion transfer process.

In this method a latent image is formed in a photographic material having a gelatino silver halide light-sensitive layer, usually a silver chloride layer. The latent image is developed in the presence of a solvent for the silver halide and while the material is in face contact with a so-called "reception sheet." The reception sheet is normally not itself light-sensitive, but it includes a surface layer containing a substance which will constitute nuclei for the photographic development process. When the layers are peeled apart the reception sheet is found to carry a positive record in developed silver of the original image.

It is believed that the result is obtained because some of the silver halide in the areas not carrying the latent image dissolves in the silver halide solvent or forms a complex therewith and diffuses into the reception sheet where, in association with the development nuclei present in that sheet and in the presence of the developing substance, it develops to form an image in that sheet.

The method is described in British Patent No. 614,155, French Patent No. 879,995, and other patent literature, and is practised widely on a commercial scale for document reproduction. As stated above, it is known as the "diffusion-transfer" process and for the sake of brevity it will be so described herein.

It is a difficulty with the said process that the color of the image obtained in the reception sheet tends, in the absence of any toning agent specially present, to be a somewhat unsatisfactory brown in color, whereas for both aesthetic reasons and for reasons of establishing a high contrast between image and background, as nearly black an image as possible is preferred.

Various proposals have been made to provide that the positive image should be of improved color, and in this connection reference may be made to British Patent No. 695,905 which proposes the use of a mercapto tetrazole for the purpose. However, extensive experiment has failed to reveal any relation between the various compounds which will improve the image colour such as would enable any hypothesis to be set up as to the type of compound which will be effective. Indeed, the matter must still be treated on a wholly empirical basis.

It has now been found, and this forms the basis of the present invention, that a particular narrow class of pyrazolenine derivative is effective for the purpose indicated.

According to the present invention, therefore, in the diffusion-transfer process of photographic reproduction, the development of the latent image in the silver halide emulsion layer is effected in the presence of a compound of the general formula:



where R and R' are alkyl groups, preferably lower alkyl groups such as methyl or ethyl, or together form a 5-membered or 6-membered saturated ring, and X is an alkyl, e.g. methyl or ethyl, aralkyl, e.g. benzyl, alkylthio,

2

e.g. methylthio or ethylthio, or alkoxy, e.g. ethoxy or methoxy group.

The following are typical compounds of the aforesaid general formula with this method of production:

### A. 3-MERCAPTO-4:4:5-TRIMETHYL-PYRAZOGENINE

Ethyl  $\alpha$ - $\alpha$ -dimethylacetacetate (15.8 g.) and 90% hydrazine hydrate (5.8 g.) were heated under reflux for three hours on a steam bath. Ethanol and water were then removed by evaporation under reduced pressure and the residual oil rapidly crystallised. Recrystallisation from benzene-light petroleum yielded fine colourless needles of pure 4:4:5-trimethyl-3-pyrazolone, M. Pt. 108° C.

4:4:5-trimethyl-3-pyrazolone (30 g.) was dissolved in dry xylene (150 cc.) and finely powdered fresh phosphorous pentasulphide (53 g.) added with stirring. The mixture was then stirred and refluxed for one hour, cooled, and mixed with ice (500 g.). After leaving for sixteen hours at room temperature the mixture was extracted with benzene (3 x 200 cc.) and evaporation of the combined benzene solutions left a yellow crystalline mass. This solid was recrystallised from water to yield 3-mercaptop-4:4:5-trimethylpyrazolene as fine pale yellow needles, M. Pt. 112° C.

The aforesaid compound is the preferred compound for use in the diffusion-transfer process in accordance with the present invention.

### B. 3-MERCAPTO-4:4-DIETHYL-5-METHYL-PYRAZOGENINE

4:4-diethyl-5-methyl-3-pyrazolone was obtained by reaction of ethyl  $\alpha$ - $\alpha$ -diethylacetacetate (20 g.) and hydrazine hydrate (5.3 g.) and crystallised from light petroleum as colourless crystals, M. Pt. 103-108°.

4:4-diethyl-5-methyl-3-pyrazolone (2.7 g.), xylene (49 ml.) and phosphorous pentasulphide (4.2 g.) were boiled under reflux for two hours, cooled, and diluted with water (122 ml.). The xylene and some of the water were removed by distillation under reduced pressure and the residual solution was cooled to precipitate the product. Recrystallisation from water in the presence of decolorising charcoal gave the product as yellow needles, M. Pt. 140-143°.

### C. 4:5-DIMETHYL-4-ETHYL-3-MERCAPTO-PYRAZOGENINE

Ethyl  $\alpha$ -ethyl- $\alpha$ -methyl acetacetate (James, Annalen 1884, 226, 209) (33 g.) and 90% hydrazine hydrate (9.6 g.) were heated on a steam bath for 3 hours. Xylene (100 ml.) was added to the solution and the solution distilled at atmospheric pressure until all the ethanol and water had been removed. The solution was filtered and, on standing, 4:5-dimethyl-4-ethylpyrazol-3-one crystallised as colorless needles, M. Pt. 76-77° C.

55 The mercapto compound was prepared from this intermediate by the method given for 3-mercaptop-4:4:5-trimethylpyrazolene, and crystallised from water as pale yellow needles, M. Pt. 80-82° C.

### D. 5-BENZYL-4:4-DIMETHYL-3-MERCAPTO-PYRAZOGENINE

5-benzyl-4:4-dimethylpyrazol-3-one was prepared from hydrazine and ethyl  $\alpha$ - $\alpha$ -dimethyl- $\gamma$ -phenylacetacetate (Blaise, Compt. Rendus, 1901, 132, 480) and obtained from aqueous solution as colorless needles, M. Pt. 116-118°.

5-benzyl-4:4-dimethylpyrazol-3-one (8 g.) and fresh powdered phosphorus pentasulphide (20 g.) and xylene (200 ml.) were heated under reflux for one hour. The xylene solution was poured on to ice (200 g.) and left for 16 hours. The aqueous suspension was extracted with benzene and the benzene solution was evaporated to dry-

ness, leaving a red oil. The oil was warmed with 5% sodium carbonate solution and the insoluble portion was filtered off. On adjusting the solution to pH 9 with dilute hydrochloride acid, the product crystallised as yellow needles, M.Pt. 118-120° C.

**E. 3-MERCAPTO-5-METHYL-4:4-CYCLOPENTA-METHYLENEPYRAZOLENINE**

5-methyl-4:4-cyclopentamethylenepyrazol - 3 - one was prepared from hydrazine and ethyl 1-acetylcylohexane-carboxylate (Braun, Berichte, 1907, 40, 3944) was crystallised from aqueous solution as colorless needles, M.Pt. 127-129°.

3 - mercapto - 5 - methyl - 4:4 - cyclopentamethylene-pyrazolenine was prepared from this intermediate and purified by the method given for 5-benzyl-4:4-dimethyl-3-mercaptopypyrazolenine. It was obtained as yellow needles, M.Pt. 132-134° C.

Any of the compounds of the general formula given above can usefully be added to the developer employed in the diffusion transfer process in quantities of, for example, 0.02 g. to 0.5 g./litre. It can alternatively be included in the photographic emulsion itself, e.g. in a proportion of 0.01 g. to 0.5 g./litre of emulsion coated, or it may be included in the reception sheet, e.g. in a proportion of 0.02 to 2 g./litre of the coating solution applied to the reception sheet. Alternatively, quantities of the compound of the order indicated may be distributed as between the developer, emulsion and reception sheet, or any two of these. In a further variant the photographic material or the reception sheet may be wetted with a solution of the compound as a pre-treatment before being subjected to the developing process.

The following examples will serve to illustrate the invention:

*Example 1*

A reception sheet was coated with a 5% (w./v.) solution of gelatin containing 0.025 g. of colloidal silver sulphide, 20 g. of sodium thiosulphate and 0.2 g. of 3-mercaptop-4:4:5-trimethylpyrazolenine per litre. A silver chlorobromide emulsion coated on paper was exposed and both the reception sheet and the exposed sheet were impregnated with a developer of the following composition:

|                                     | G.  |
|-------------------------------------|-----|
| Sodium sulphite (cryst.)            | 100 |
| Hydroquinone                        | 10  |
| p-Methyl amino phenol hydrochloride | 2   |
| NaOH                                | 10  |
| KBr                                 | 0.5 |
| Water to 1 litre.                   |     |

The two layers were pressed together and separated after one minute. The reception layer carried a neutral-toned positive image.

*Example 2*

A silver chlorobromide emulsion coated on paper was exposed and, together with a reception sheet of the type described in Example 1 but not containing the pyrazolenine compound, was impregnated with a developer of the following composition:

|                                         | G.  |
|-----------------------------------------|-----|
| Sodium sulphite (cryst.)                | 100 |
| Hydroquinone                            | 10  |
| p-Methyl amino phenol sulphate          | 2   |
| NaOH                                    | 10  |
| KBr                                     | 0.5 |
| 3-mercaptop-4:4:5-trimethylpyrazolenine | 0.3 |
| Water to 1 litre.                       |     |

The two layers were pressed together and separated after one minute. The reception layer carried a neutral-toned positive image.

*Example 3*

A silver chlorobromide emulsion containing 0.5 g. per litre of 3 - mercapto - 4:4:5 - trimethylpyrazolenine was

coated on paper. The coating was then exposed and, together with a reception sheet of the type described in Example 1 but not containing the pyrazolenine compound, was impregnated with a developer of the following composition:

|                                | G.  |
|--------------------------------|-----|
| Sodium sulphite (cryst.)       | 100 |
| Hydroquinone                   | 10  |
| p-Methyl amino phenol sulphate | 2   |
| NaOH                           | 10  |
| KBr                            | 0.5 |
| Water to 1 litre.              |     |

The two layers were pressed together and separated after one minute. The reception layer carried a neutral-toned positive image.

When, in the foregoing examples the specified pyrazolenine compound is replaced by any other of the pyrazolenine compounds specifically set forth above, in equal amount, similar results are obtained.

20 What we claim is:

1. A method for the production of photographic records from silver halide photographic emulsions by the diffusion transfer process which comprises developing a photographic silver halide emulsion layer while the emulsion layer is in face contact with a layer containing development nuclei, the development being effected in the presence of a solvent for silver halide and a compound of the general formula:



30 wherein R and R' taken separately represent alkyl groups and taken together represent a saturated ring containing at least 5 and at most 6 members in the ring, and X represents a group selected from the class consisting of alkyl, aralkyl, alkylthio and alkoxy groups.

40 2. A method for the production of photographic records from silver halide photographic emulsions by the diffusion transfer process which comprises developing a photographic silver halide emulsion layer while the emulsion layer is in face contact with a layer containing development nuclei, the development being effected in the presence of a solvent for silver halide and 3-mercaptop-4:4:5-trimethylpyrazolenine.

45 3. A method for the production of photographic records from silver halide photographic emulsions by the diffusion transfer process which comprises developing a photographic silver halide emulsion layer while the emulsion layer is in face contact with a layer containing development nuclei, the development being effected in the presence of a solvent for silver halide and 3-mercaptop-4:4-diethyl-5-methylpyrazolenine.

50 55 4. A method for the production of photographic records from silver halide photographic emulsions by the diffusion transfer process which comprises developing a photographic silver halide emulsion layer while the emulsion layer is in face contact with a layer containing development nuclei, the development being effected in the presence of a solvent for silver halide and 4:5-dimethyl-4-ethyl-3-mercaptopypyrazolenine.

60 65 5. A method for the production of photographic records from silver halide photographic emulsions by the diffusion transfer process which comprises developing a photographic silver halide emulsion layer while the emulsion layer is in face contact with a layer containing development nuclei, the development being effected in the presence of a solvent for silver halide and 5-benzyl-4:4-dimethyl-3-mercaptopypyrazolenine.

70 6. A method for the production of photographic records from silver halide photographic emulsions by the diffusion transfer process which comprises developing a photographic silver halide emulsion layer while the emulsion layer is in face contact with a layer containing de-

development nuclei, the development being effected in the presence of a solvent for silver halide and 3-mercaptop-5-methyl-4:4-cyclopentamethylenepyrazolenine.

7. A method for the production of photographic records from silver halide photographic emulsions by the diffusion transfer process which comprises developing a photographic silver halide emulsion layer while the emulsion layer is in face contact with a layer containing development nuclei, the development being effected in the presence of a solvent for silver halide and the emulsion containing 0.01 to 0.5 g./litre of emulsion coating of a compound of the general formula:



wherein R and R' taken separately represent alkyl groups and taken together represent a saturated ring containing at least 5 and at most 6 members in the ring, and X represents a group selected from the class consisting of alkyl, aralkyl, alkylthio and alkoxy groups.

8. A method for the production of photographic records from silver halide photographic emulsions by the diffusion transfer process which comprises developing a photographic silver halide emulsion layer while the emulsion layer is in face contact with a layer containing development nuclei, the development being effected in the presence of a solvent for silver halide and the developer containing 0.02 to 0.5 g./litre of a compound of the general formula:



wherein R and R' taken separately represent alkyl groups and taken together represent a saturated ring containing at least 5 and at most 6 members in the ring, and X represents a group selected from the class consisting of alkyl, aralkyl, alkylthio and alkoxy groups.

9. A method for the production of photographic records from silver halide photographic emulsions by the diffusion transfer process which comprises developing a photographic silver halide emulsion layer while the emulsion layer is in face contact with a layer containing development nuclei, the development being effected in the presence of a solvent for silver halide and the layer containing the development nuclei further containing 0.02 to 2 g./litre of the coating applied of a compound of the general formula:



wherein R and R' taken separately represent alkyl groups and taken together represent a saturated ring containing at least 5 and at most 6 members in the ring, and X represents a group selected from the class consisting of alkyl, aralkyl, alkylthio and alkoxy groups.

10. A photographic silver halide emulsion containing a compound of the general formula:



15. wherein R and R' taken separately represent alkyl groups and taken together represent a saturated ring containing at least 5 and at most 6 members in the ring, and X represents a group selected from the class consisting of alkyl, aralkyl, alkylthio and alkoxy groups the said compound being present in a proportion of 0.01 to 0.5 g. per litre of emulsion coated.

20. 11. A photographic developer composition containing a silver halide solvent and 0.02 to 0.5 g. per litre of a compound of the general formula:



wherein R and R' taken separately represent alkyl groups and taken together represent a saturated ring containing at least 5 and at most 6 members in the ring, and X represents a group selected from the class consisting of alkyl, aralkyl, alkylthio and alkoxy groups.

25. 12. An element for use in photography comprising a support carrying a layer which includes photographic development nuclei and a compound of the general formula:



30. 40. wherein R and R' taken separately represent alkyl groups and taken together represent a saturated ring containing at least 5 and at most 6 members in the ring, and X represents a group selected from the class consisting of alkyl, aralkyl, alkylthio and alkoxy groups the said compound being present in a proportion of 0.02 to 0.2 g. per litre of the coating solution applied to form said layer.

45. 55. References Cited in the file of this patent

UNITED STATES PATENTS

2,699,393 Weyde ----- Jan. 11, 1955